

# United States Patent Office

2,824,829

Patented Feb. 25, 1958

1

2,824,829

## ELECTRODEPOSITING BLACK CHROMIUM-VANADIUM COATINGS AND MEMBERS THEREWITH

Martin F. Quaely, Montclair, N. J., assignor to Westinghouse Electric Corporation, East Pittsburgh, Pa., a corporation of Pennsylvania

No Drawing. Application June 8, 1956  
Serial No. 590,113

4 Claims. (Cl. 204—43)

This invention relates to the electrodeposition of black coatings of chromium and vanadium.

This application is a continuation-in-part of my application Serial No. 339,469, filed February 27, 1953, now abandoned, and assigned to the assignee of the present invention.

It has been desirable to electrodeposit black coatings on members. Black coatings are desirable for decorative and similar applications, as for instance in making name plates and the like. However, there is a particular need in the electronic industry for black coatings that have adherence and stability when exposed to elevated temperatures especially under high vacuum conditions.

The object of this invention is to provide a process for electroplating on members a black coating comprising a complex of chromium and vanadium.

A further object of the invention is to provide members having an applied adherent black coating comprising a complex of chromium and vanadium.

Another object of this invention is to provide an electrolyte comprising an aqueous solution of a chromium compound, a vanadium compound and an organic carboxyl acid, such that black coatings may be electrodeposited from said electrolyte upon members.

Other objects of the invention will in part be obvious and will in part appear hereinafter.

I have discovered a process for depositing novel black coatings on members, the coatings characterized by high stability and adherence to members even when heated to temperatures of 750° C. while in a vacuum. The process comprises the preparation of an aqueous electrolyte comprising essentially (a) from 150 to 385 grams per liter of chromic acid, (b) from 1.8 to 10 grams of vanadium in a soluble compound thereof, the latter being supplied, for example, as from about 4 to 23 grams per liter of ammonium metavanadate, there being present from 100 to 9.5 parts by weight of chromium per part of vanadium, and (c) from 3 to 20 grams per liter by weight of a water soluble carboxylic acid.

Exceptionally good results have been obtained from electrolytes containing 200 grams per liter of chromic acid ( $\text{CrO}_3$ ), and 20 grams per liter of ammonium vanadate. The ratio of chromium to vanadium in this electrolyte is 11.9 to 1.

The vanadium compound may comprise ammonium metavanadate, a vanadium halide or other vanadium compound soluble in water in the required proportions. Metallic vanadium powder or solid vanadium metal may be dissolved in concentrated nitric acid to produce a soluble vanadium compound for the purpose of the invention. Mixtures of two or more vanadium compounds may be employed in the electrolyte.

Examples of suitable water soluble carboxylic acids are acetic acid, formic acid, citric acid, oxalic acid and propionic acid and mixtures of any two or more thereof.

The aqueous electrolyte so prepared is disposed in an electroplating tank or cell, resistant to the action of chromic acid solutions. Glass, ceramic or rubber lined

2

tanks are suitable for this purpose. The electrolytic cell should be provided with suitable cooling means in order to maintain the temperature of the electrolyte within the range of approximately 30° C. to 50° C. Members to be plated are made the cathode in the cell while the anode comprises lead plates. However, carbon or graphite anodes or anodes of other insoluble materials commonly used in chromium plating may be employed. The member to be plated will ordinarily comprise a metallic body, but other materials than metals may be plated after first applying thereto a conductive coating such, for example, as graphite or chemically precipitated silver. A potential of from 12 to 15 volts is applied between the cathode and the anode and a current density of from 400 to 2,000 amperes per square foot is passed through the cathode. The composition of the bath is maintained by the addition of the chromium and vanadium compounds as they become used up during the plating operation. Small amounts of mineral acids are tolerated by the bath though ordinarily the electrolyte is kept free of any extraneous additions.

The following examples illustrate the practice of the present invention:

### Example I

There was placed in a glass plating cell an aqueous electrolyte comprising 200 grams per liter of chromic acid ( $\text{CrO}_3$ ), 10 grams per liter of ammonium metavanadate, and 6½ milliliters of glacial acetic acid. A steel plate was made the cathode in the electrolyte with a lead plate being the anode. An electrical current at a density of 900 amperes per square foot was applied to the steel member. In 5 minutes' plating, a black coating of a thickness of approximately 1 mil was deposited on the steel plate. The steel plate was then removed from the electrolyte and washed with water. The applied black coating was found to be very adherent to the steel plate. When heated in a vacuum to temperatures of 750° C., the color of the coating remained unchanged. When heated in an oxidizing gas flame, the color of the coating changed from a jet black to a gray black.

### Example II

An electroplating electrolyte similar to that of Example I was prepared. A copper anode-support such as is used in a rotating anode X-ray tube was made the cathode after having been previously cleaned to remove surface oxides. The copper anode-support was plated in the electrolyte at a current density of 1,000 amperes per square foot for 5 minutes. The anode-support was provided with a jet black coating of a thickness of approximately 1 mil. The anode-support was then assembled with the tungsten anode and was next placed in an X-ray tube which was thereafter sealed and evacuated. The tube was then put into operation and the anode rotated at a speed of 3,600 R. P. M. and subjected to an electron beam to produce X-rays therefrom. The coating was found to have a high thermal emissivity. The electrodeposited black coating was found to be highly adherent and unimpaired by longtime use.

### Example III

An electrolyte is prepared by dissolving 384 grams per liter of chromic oxide ( $\text{CrO}_3$ ) and 4.6 grams per liter of ammonium vanadate. To each liter of the solution is added 5 milliliters of glacial acetic acid. Adherent jet black coatings are electrodeposited on members by plating at current densities of 800 amperes per square foot applied for 5 minutes, the electrolyte being at 35° C.

Many members and structures may be provided with the electrodeposited black coatings of this invention. Thus, parts of electrical appliances, electronic devices and radia-

tion emitting devices may be coated to provide thereon the black coatings to improve their operation or for decorative or other purposes.

Analysis indicates that the black electrodeposits comprise chromium and vanadium in substantially the same proportion as in the electrolyte, that is, the coatings comprise from 100 to 9.5 parts by weight of chromium per part of vanadium. The black coatings comprise both the metals and the oxides of chromium and vanadium. Spectroscopic and other analysis shows that the vanadium is present primarily as vanadium trioxide ( $V_2O_3$ ) with only a small portion of vanadium metal, and that the chromium is primarily present as metal with only a small proportion of chromium oxide. In the black coatings of the chromium-vanadium-oxygen complex there are present from 100 to 2 atoms of chromium per oxygen atom combined therewith.

It is intended that all matter contained in the above description shall be deemed to be illustrative and not limiting.

I claim as my invention:

1. An aqueous electroplating electrolyte comprising essentially from 150 to 385 grams per liter of chromic acid, from 1.8 to 10 grams per liter of vanadium in soluble compound form, there being present from 100 to 9.5 parts by weight of chromium per part of vanadium, and from 3 to 20 grams per liter of a water soluble carboxylic acid.

2. An aqueous electroplating electrolyte comprising essentially from 150 to 385 grams per liter of chromic acid, from 4 to 23 grams per liter of ammonium vanadate, and from 3 to 20 grams per liter of a carboxylic acid selected from the group consisting of acetic acid, citric acid, formic acid, oxalic acid and propionic acid.

3. In the process of electrodepositing an adherent highly heat-resistant black finish on a member, the step comprising making the member a cathode in an aqueous electroplating electrolyte comprising essentially from 150 to 385 grams per liter of chromic acid, from 1.8 to 10 grams per liter of vanadium in soluble compound form, there being present from 100 to 9.5 parts by weight of chromium per part of vanadium, and from 3 to 20 grams per liter of a water soluble carboxylic acid, and passing a plating electrical current through the member at a current density of from 400 to 2,000 amperes per square foot, the electrolyte being maintained at a temperature of from 30° C. to 50° C.

4. A member having on its surface an adherent, highly heat resistant, black coating consisting of chromium, vanadium and oxygen, the vanadium being present primarily as vanadium trioxide and the chromium primarily as metallic chromium with a minor proportion of chromium oxide, there being a total of from 100 to 2 atoms of chromium per atom of oxygen combined therewith, and from 100 to 9.5 parts by weight of chromium per part by weight of vanadium.

#### References Cited in the file of this patent

#### UNITED STATES PATENTS

|           |                 |               |
|-----------|-----------------|---------------|
| 1,542,549 | Grah            | June 16, 1925 |
| 4,795,459 | Westbrook       | Mar. 10, 1931 |
| 4,975,239 | Ungelenk et al. | Oct. 2, 1934  |
| 2,623,847 | Gilbert et al.  | Dec. 30, 1952 |

#### OTHER REFERENCES

Jones: Powder Metallurgy, 1943, pp. 154-4.